

C. VICKERS.

MEANS FOR CASTING METALS, INCLUDING THEIR ALLOYS.  
APPLICATION FILED AUG. 29, 1914.

1,172,506.

Patented Feb. 22, 1916.



Witnesse<sup>s</sup>  
S. A. Jarry  
Philadelphia

Inventor  
Charles Dickens.  
By Walter D. Edmunds  
attorney

# UNITED STATES PATENT OFFICE.

CHARLES VICKERS, OF NIAGARA FALLS, NEW YORK, ASSIGNOR TO THE TITANIUM ALLOY MANUFACTURING COMPANY, OF NEW YORK, N. Y., A CORPORATION OF MAINE.

## MEANS FOR CASTING METALS, INCLUDING THEIR ALLOYS.

1,172,506.

Specification of Letters Patent. Patented Feb. 22, 1916.

Application filed August 29, 1914. Serial No. 859,156.

To all whom it may concern:

Be it known that I, CHARLES VICKERS, a subject of the King of Great Britain, and a resident of Niagara Falls, in the county of Niagara and State of New York, have invented certain new and useful Improvements in Means for Casting Metals, Including Their Alloys, of which the following is a specification.

10 My present invention relates to the casting of metals, and, particularly, of certain of their alloys, and its objects comprise provision of a method whereby, by aid of the novel means herein described and 15 claimed, the tensile strength, ductility, homogeneity, purity, and other desirable properties, of the resulting castings may be enhanced in a manner more simple, economical, and certain than heretofore known 20 or practised for such purposes.

It seems now established that the characteristics of metals, and especially of certain alloys thereof, may be, more or less, and sometimes controllingly, affected by so-called "heat-treatments," i. e., applications thereto of various specific temperatures designedly produced, or maintained, prior to, during, or after, casting. These phenomena seem attributable to physical changes, or 30 also chemical reactions between, constituents of the metallic mass, which are inaugurated, or promoted, or hindered, as the case may be, by various specific temperatures, or their duration, and are often evidenced by 35 resulting variations in grain, size of crystals, etc., and also, and in alloys more frequently, by formation, or reduction, of divers chemical compounds during the operation. Acceptance of such doctrines has resulted in resort by manufacturers to many 40 troublesome, expensive, and more or less inefficient expedients, in hopes of thereby satisfactorily creating, adjusting, regulating, maintaining, varying, or controlling, 45 at various times and stages, the temperatures of the metals operated on, such being, for example, attempts to secure certain specific temperatures during pouring, attempts to delay, or otherwise vary, the temperatures 50 during solidification as by pre-heating the molds, or by quenching, in water, the released casting and even after its solidification as by annealing, or heating and slowly

cooling it, etc. A good example of such expedients and their results is afforded by 55 the subsequent treatment accorded to manganese steel castings, the annealing and quenching of which has great influence on their physical properties. Therefore, in industrial practice, good foundry men in casting different metals and their alloys have felt obliged to pay particular attention to the nature of each, to its temperature in the ladle, to its temperature in the molds which may, or not, require cautious heating, to the 60 creation, maintenance, limitation, or reduction of temperatures during cooling, etc. etc.; but, notwithstanding their greatest care and skill their final products have hitherto too often been marred by characteristics rendering them so unsuitable for the purpose intended, as to necessitate additional expensive and uncertain heat-treatments in further, often equally fruitless, endeavors to thus doctor them up to standard 70 requirements. The hitherto unavoidable uncertainty of producing castings of prescribed quality and characteristics has, in short, prior to my invention, proved detrimental to the art, because of the numerous 75 factors entering into the problem, and the resulting expense of even approximately solving their required proper bearing on each batch of metal treated. The result has been that castings hitherto obtainable in 80 market, including particularly those of alloyed metals, have too often proved undesirably weak, or otherwise imperfect, owing to segregation, porosity, lack of homogeneity, impurities, and other defects attributable, largely, if not entirely, to substantially 85 unavoidable, imperfect, or insufficient, regulation, or control, of the temperature factors during their manufacture on industrial scales. 95

The object of my present invention comprises provision of a method, and means for its practice, whereby castings of metals, and particularly of their more difficultly treated alloys, may be manufactured under usual 100 industrial conditions, with less expense than heretofore, with less technical skill and attention on the part of the operators, and with much greater certainty of final products possessing better qualities including 105 greater purity and homogeneity, less segre-

gation and porosity, and consequent superior ultimate strength, elongation and reduction.

I attain my object by my hereinafter described method and means for its practice.

I have discovered that requisite "heat-treatment", or regulation, of the temperatures of castings can be, and is, most readily, economically, certainly, and efficiently, applied in all cases by merely correspondingly regulating the composition, or constituents, of the molds, thus confining all heat-treatment to the period, or stage, of therein cooling. I am thereby enabled to dispense with all heatings other than required to qualify the metal for pouring, and with all quenchings, or coolings, other than administered through the agency of the constituents of the mold. I have also discovered that final products whose temperatures during production have been thus regulated and sufficiently controlled and varied by aid of no other medium than that afforded by appropriately selected, prepared, and proportioned integral constituents of the mold itself, are in all desirable characteristics vastly superior to any hitherto known to me including those improved as much as possible by any heretofore practised "heat-treatments" either before, during, or after the casting. I have further discovered that my aforesaid system of heat-treating, during the cooling of the metal, in the mold itself, is usually productive of the best results when applied in a particular manner, *i. e.* by the use of certain non-metallic, specific, substances, or mixtures, as constituents of the mold, and by their special dispositions and arrangements relatively to each other as hereinafter exemplified.

I am satisfied that, among others, one of the most frequent causes of faulty castings, particularly in the case of alloys, is the "liquation" attributable to too slow cooling of the metal in the mold. It has thus, heretofore, too frequently happened that in the production of castings from alloys comprising two metals, the one of which is of high, and the other of relatively low, melting point, a separation throughout the casting into alloys of differing composition takes place. Those of such alloys having the highest fusing point solidify first and the entire mass becomes only gradually solid by further cooling. Thus when "freezing" or solidification commences, an alloy rich in the metal of the higher melting point and poor in the metal of the lower melting point, will first separate as a solid, and this is followed by the solidification of various other alloys containing progressively less of the former metal and more of the latter, the last alloy to separate and solidify being proportionately very rich in the metal of lower melting point, and correspondingly poor in

the other; this being known as the "eutectic alloy". The resulting casting is correspondingly lacking in homogeneity, is not throughout uniform in composition, and is consequently weaker, in spots, than it should be. I have found that this liquation, and its injurious effects on the product are greatly, or altogether, preventable by chilling the metals, while in the mold, much more rapidly than I believe has hitherto been industrially known or attempted. Homogeneity in the molten alloy as regards its constituent metals is by present well known practice sufficiently attainable and maintainable up to the time of its pouring into the mold. It is in the latter that the undesired noxious liquation occurs. It is there that it must, if possible, be obstructed or prevented, and this I accomplish by there contacting the molten casting with the most rapidly heat-conductive, or diffusive, substance which I have yet found adapted to the purpose, to wit, graphitized carbon, and usually preferably in the form known as "artificial graphite". To this end I construct the mold principally of said substance which is also advantageous for the purpose for the additional reasons that it contains substantially no moisture, and no gases for the molten metal to absorb, all volatile matter having been expelled therefrom by the high temperatures required for its production, as, for example, usually those of the electric furnace. It is also so extremely refractory, and resistant of high temperatures, as to correspondingly impart permanence to the forms composed in whole, or in part, thereof, thus enabling the use of molds containing it to be correspondingly indefinitely repeated.

My present invention therefore comprises the construction of the molds in such manner as to thereby regulate the cooling to normal temperatures of the therein molten metal at such rates as indicated by its nature and constituents and the obtaining of the best resultant castings.

My researches have demonstrated that, as a rule, not only prevention of liquation, but also the all-around perfection and excellence of the casting is proportional to the rapidity of its cooling, while it remains *in situ* in the mold, and that such rapidity, in the high degree required, is best, most practically, and least expensively attainable by the influence, or through the medium of, a constituent substance of the mold preferably disposed so as to contact, and thus assist in the shaping of the casting.

It is presumable that mere acceleration of chill, or solidification, might be imparted by resort to other means or agents, as for example by auxiliary water-cooling devices, or an air-blast, but these, in addition to other practical objections, are not only com-

paratively expensive and difficult of proper application, but they are incapable of producing the same desired influence on, and results in, the metal, as are obtainable through the rapidity imparted by the high heat-conductive, or diffusive, properties of the molding material itself. Again, although I have found that many substances, as, for example, metals, and particularly iron, are more rapidly heat-conductive than the sand so generally used in molding; the iron molds hitherto essayed have proved unsatisfactory for many reasons, including their too frequently deleterious effects on the molten metals, their comparative cumbersomeness, the difficulty of producing and manipulating them as required, and especially their incapacity to afford that relatively accurate and uniform adjustment of the locally, and otherwise varying, heat-withdrawing properties of my molds which is of importance to the most successful practice of my method.

I have thus far, as above stated, found no other substance so well adapted to the purposes of my invention as is graphitized carbon. This substance, in addition to its above enumerated favorable qualities, is capable of having its heat-conductive property readily modified and thus adjusted to meet the requirements of different metals, or even different parts of the same casting. For example, I have, to meet some requirements, constructed my permanent molds by mixing graphite, either artificial or natural, with any suitable binder such as tar or pitch, forming it by usual procedures into the proper shape and then baking it in a furnace as in ordinary carbon manufacture. If by this procedure a heat-conductivity is imparted to the mold too great for successful use in certain forms of castings, I have adjusted the heat-conductivity to that required by adding to the constituent mixture a certain amount of amorphous carbon determined to be sufficient to sufficiently reduce, for the special purpose, the heat-conductivity of the mold.

I can also form my permanent molds wholly out of amorphous carbon and then graphitize them in an electric furnace. Here, again, I am able to adjust as required their heat-conductivity; for by correspondingly adjusting the temperature of the furnace I am, as will be well understood, able to regulate the extent of the graphitization, or the polymerization, of the amorphous carbon, and thus correspondingly control the heat conductivity of the resulting mold. I can also further locally adjust the heat-conducting properties of my permanent molds, by varying their thickness at different points, or zones, corresponding with the thicker and thinner parts of the casting, and, by this means, readily insure more

rapid heat-withdrawal from the thicker parts, and less rapid from the thinner, thus insuring substantial uniformity of heat-withdrawal from all parts of the casting at the same rate and in equal amount during a given time.

In cases wherein a permanent mold is not desired or required, I construct a temporary mold such as employed in making many forms of castings. For this purpose if the mold, as rarely if ever happens, is to be composed entirely of graphite, I merely form that substance to the desired pattern under high pressure, as will readily be understood, and in such instances I have found that the best form of graphite for the purpose is that obtained by the well known decomposition of silicon carbide, or other like carbides, since this form possesses plastic coherent properties when subjected to pressure. Or, as more frequently demanded, I make the temporary mold as last aforesaid, but out of a mixture of graphitized carbon and ordinary molder's sand regulating the proportions so as to impart to the mold the degree of heat-conductivity best suited to the particular kind of casting desired. In such cases I can also, as in the above referred to examples of my permanent molds, locally vary and adjust the heat-conductivity of different parts of the mold by correspondingly increasing, or diminishing, the proportion of sand in the mixture at those localities. The comparative merits of my invention have been repeatedly demonstrated.

In one instance, designed particularly to show the influence of my aforesaid methods of rapid cooling on the physical properties of the castings, I employed an alloy containing 92 per cent. of aluminum and 8 per cent. of copper. From this alloy I made castings from the same heat in four different molds made respectively of sand, amorphous carbon, iron, and graphitized carbon. Tests of the physical properties of the resulting castings gave the respective results indicated by the subjoined table, viz:—

| Casting.                        | Ultimate strength. | Per cent. elongation. | Per cent. reduction. | 115 |
|---------------------------------|--------------------|-----------------------|----------------------|-----|
| In sand mold.....               | 12,300             | 1.0                   | 0.7                  |     |
| In amorphous carbon mold.....   | 17,700             | 1.8                   | 1.3                  |     |
| In iron mold.....               | 25,500             | 3.5                   | 4.1                  |     |
| In graphitized carbon mold..... | 26,300             | 3.8                   | 4.4                  | 120 |

The four substances thus employed are superior to each other in heat-conductivity as molds in the order named, that of sand being much the least, and that of graphitized carbon the greatest.

Similar tests made with other alloys gave analogous results.

Again tests made of the efficiency of my above referred to temporary molds made of

a mixture of sand with graphite, as compared with that of sand molds in casting the said alloy of 92 per cent. aluminum and 8 per cent. copper gave the following results:

| Casting.                      | Ultimate strength. | Per cent. elongation. | Per cent. reduction. |
|-------------------------------|--------------------|-----------------------|----------------------|
| From sand mold .....          | 21,650             | 2.5                   | 2.7                  |
| From graphite-sand mold ..... | 26,780             | 4.0                   | 4.7                  |

I have furthermore discovered that a mold composed entirely of graphitized carbon only is, by itself alone, incompetent to impart, in highest degree, to the castings, the above noted improved physical characteristics. My researches have demonstrated that to attain these more universally, and perfectly, than otherwise possible, there is required, in the mold, a combination of the rapidly heat-diffusing substance with another comparatively much less so. This, I have discovered, is important for several reasons, as, for example, the need of providing means to overcome the effects of natural shrinkages and contractions of the metal, which render it desirable, during solidification, to constantly supply thereto additions thereof, which are, at the time, so comparatively liquid as to be capable of flowing into cavities caused by contractions of the original charge and thus restore thereto its required bulk. Again, as above referred to, some sections of a given casting may require more rapid cooling than others, in order that the casting, as a whole, may solidify at a uniform rate. This, as will be understood, is the case when a casting consists of alternate thin and heavy sections, in which event graphitized carbon is preferable to form the mold walls around the heavy sections, and some less rapidly heat-diffusing substance such as molding sand, amorphous carbon, alundum, alumina, or a mixture thereof as aforesaid with graphitized carbon, is preferable around the thinner sections.

My molds may therefore be made either entirely or, preferably only principally, of the more rapidly heat diffusing substance. In the latter case, I use that substance as aforesaid, per present methods of constructing a sand-mold, of which it may thus form a part; or, in cases in which my aforesaid combination of substances is relied on to also overcome undesired results of contraction, I employ the less rapidly heat diffusing, or conductive, substance as the constituent of the "feeder," or "riser," portion of the mold proper. This riser constitutes a reservoir for metal in excess of that required to first fill the mold, and is disposed, preferably, so as to communicate with the highest point of the casting in such manner that such excess metal can flow by gravity down into the mold to fill the cavities therein

quickly formed by my rapid cooling thereof, or by escape of gases therefrom through the comparatively traversable less solidified contents of the riser.

For a better understanding of my invention, generally, and as typical of constructions last referred to, I have diagrammatically illustrated my combination of a more heat-conductive mold, with a less heat-conductive riser in the accompanying drawings in which—

Figure 1 is a top, or plan, view of such combination and Fig. 2 a vertical section on the line 2—2 of Fig. 1.

Referring to these, A is the body of the mold for the casting proper, having, as shown by the drawings, the bottom and sides of its matrix composed, in this instance, of the more rapidly heat-conducting substance or mixture, and B is its riser, lined, in the usual manner, with a less rapidly heat-conducting substance, or mixture, as, for example, ordinary molders' sand packed within a bottomless holder B' by ramming it therein around a therewith concentric core (not shown because necessarily withdrawn to produce the cavity for the riser). B is, as shown, disposed, preferably, on top of the carbon mold and concentrically therewith, and is thus, for the purposes of the operation, a part of the latter, the major part of the top of the matrix of which is, as shown in the drawings, covered or inclosed by solid portions of the therewith communicating riser. The mold A is, in this instance, as is preferable, provided with a therein-contained gate, or duct C, for charging the molten metal into the mold proper. This extends, as shown, from at least the level of the top of the riser to, preferably, a point C' located at the bottom of the matrix of the mold A, though it might vent into the latter at some other point. Into the upper end C<sup>2</sup> of this duct the molten metal is poured. It is conducted thereby into the mold A in which, and thence in the riser B, it ascends, in accordance with the laws governing the flow of liquids, until both are charged to the level desired. As soon as the charging has been thus completed that part of the metal designed for the casting proper, D, solidifies rapidly, influenced by the high heat-diffusive substance, or mixture, therewith in contact, while that portion of the metal located, at E, within the riser, remains relatively molten by reason of its environment by the much less heat-diffusive sand. Therefore, as the metal in D shrinks, that in E sinks into and fills the resulting cavities, thus insuring a more perfect casting than otherwise obtainable. The beneficial results of this aspect of my invention are not confined to perfectionment of the products, they produce also notable economies in the art, particu-

larly when production of massive castings is involved. This is because much less metal is required to thus "pour" a casting, fuel, time and labor being correspondingly economized, and also power in the subsequently required mechanical severing from the casting of the then therewith unitary relatively large body of surplus metal hitherto required for the riser or feeder E. This economy is directly attributable to the comparatively very rapid chilling, per my method, of the metal of the casting proper, its rate being usually many times more rapid than that of the riser. Inasmuch as only relatively small cavities form in D, thus requiring but correspondingly small additional supplies of the metal to fill them, it is, by my method, possible to successfully employ risers much smaller than heretofore relatively to the casting proper. This is because required liquidity in the riser has been heretofore maintainable, sufficiently long, only by increasing its bulk very largely in excess of that required to fill the casting. It has thus been usually necessary, in casting with sand molds for example, to have the riser fully as bulky as the casting, and in casting some alloys, such as aluminum bronze, for example, the ratio of bulk of riser to that of casting has been as high as  $1\frac{1}{2}$  to 1. But, by my method, these relative proportions of riser to casting are revolutionized, it being possible thereby to maintain, sufficiently liquid, a comparatively small riser (say, in usual practice, not to exceed one fourth the bulk of the casting), sufficiently long to supply sufficient molten metal to all cavities in the solidifying casting.

40 My method, including its employment of my molds as hereinbefore described, I have found especially advantageous in casting copper, nickel, lead, zinc, aluminum, and many alloys comprising some of those metals such as German silver, brass, bronze, "gun-metal" and "white metals", and it has proved also very useful in the casting of "ferro-metals" and their alloys.

What I claim as new and desire to secure by Letters Patent is the following, viz:— 50

1. As a new article, a mold for metal, or its alloys, composed principally of a non-metallic rapidly heat-diffusing substance, and comprising, for the casting proper, a mold composed principally of graphitized carbon, in combination with a less rapidly heat-diffusing riser. 55

2. As a new article, a mold for metal, or its alloys, composed principally of a non-metallic rapidly heat-diffusing substance, 60 and comprising, for the casting proper, a mold composed principally of graphitized carbon, in combination with a riser member composed principally of sand. 65

3. As a new article, a mold for metals, or 65 their alloys, composed partly of graphitized carbon and partly of another substance.

4. As a new article, a mold for metals, or their alloys, comprising a mixture of graphitized carbon with another substance. 70

5. As a new article a mold for metals, or their alloys, comprising a mixture containing graphitized carbon and amorphous carbon.

6. A mold for metals or their alloys having 75 the bottom and sides of its matrix composed of graphitized carbon in combination with a less rapidly heat-diffusing riser.

7. A mold for metals or their alloys having 80 the bottom and sides of its matrix composed principally of graphitized carbon, and the major portion of the top of its matrix inclosed by less rapidly heat-diffusing matter.

8. A mold for metals or their alloys having 85 the bottom and sides of its matrix composed of graphitized carbon, in combination with a less rapidly heat-diffusing riser.

9. A mold for metals, or their alloys, composed in part of graphitized carbon, and in 90 part of less rapidly heat-diffusing matter.

CHARLES VICKERS.

Witnesses:

L. E. BARTON,  
J. E. McCALLUM.